

## UNITED STATES PATENT OFFICE

2,363,301

## PRODUCTION OF MOTOR FUEL

Albert Ernest Dunstan, London, and Stanley Francis Birch, Sunbury-on-Thames, England, assignors, by mesne assignments to Anglo-Iranian Oil Company Limited, London, England

No Drawing. Original application July 27, 1937, Serial No. 155,918. Divided and this application February 18, 1941, Serial No. 379,442. In Great Britain July 29, 1936

15 Claims. (Cl. 260—683.4)

This application is a division of application U. S. Serial No. 155,918, filed July 27, 1937.

This invention relates to the production of a high class motor fuel adapted for use as an aviation or motor spirit constituent of high anti-knock rating and consisting essentially if not entirely of iso-paraffins.

According to the invention an olefine is subjected to contact with an iso-paraffin (that is a paraffin containing a tertiary carbon atom) in the presence of a mineral acid, whereby on settlement an upper hydrocarbon layer separates which is composed substantially of saturated hydrocarbons boiling within the motor spirit range from which a fully saturated aviation or motor spirit or constituent may be produced on distillation. The reaction may be carried out without the necessary use of high pressure. Thus iso-paraffins such as isobutane and isopentane and olefines such as propylene, isobutene, diisobutene and triisobutene or mixtures of such paraffins or of such olefines may be used, and the conditions of operation are advantageously such that the liquid phase is maintained during the period of contact. Furthermore, the iso-paraffins may be employed in admixture with normal paraffins which are incapable of entering into the reaction. The olefine too may be admixed with inert material. As a general rule, however, it is preferable to utilise both reactants in as pure a state as possible, since there is a tendency for the yield to be poorer and difficulties may possibly be encountered in separating the non-reactive material from the product.

According to the invention moreover the iso-paraffin or iso-paraffins may advantageously be used in substantial or considerable excess of equimolecular proportions with respect to the olefine or olefines used.

The invention comprises the process carried out under the conditions hereinafter described and the products thereof.

It is known to treat with sulphuric acid at low temperatures hydrocarbon fractions containing olefines that also contain iso-paraffins, but in such hydrocarbon fractions the content of the iso-paraffins is low, and this is the case in hydrocarbon fractions that contain lower olefines such as iso- and normal butenes suitable for use according to the invention for the production of saturated iso-paraffin derivatives boiling in the motor spirit range.

Where however equimolecular proportions of iso-butane or iso-pentane and the selected olefines react (or equivalent proportions when the

polymerides of iso-butene are used) it is necessary that substantial amounts of the iso-paraffins indicated should be made available and advantageously also isolated, in order that it may be possible for the saturated iso-paraffin derivatives to be produced according to the invention on a practical or industrial scale and under conditions of practical convenience and economy.

In carrying the invention into effect an olefine such as diisobutene is added to a mixture of an iso-paraffin such as isobutane in the presence of a mineral acid such as sulphuric acid (approximately 97 per cent), the mixture being thoroughly stirred. It is advisable that the olefine should be added gradually to the mixture while the stirring proceeds. The diisobutene is added in a ratio of one molecular proportion of diisobutene to two molecular proportions of isobutane, the isobutane being advantageously present in substantial excess of this proportion. It is advisable that the olefines should be added gradually to the mixture while the stirring proceeds. The temperature employed may ordinarily be about 0° C. In the case of isobutane however the temperature of the reaction is determined by the boiling point of the iso-paraffin which is -10.2° C. If therefore the reaction be carried out under pressure the temperature of the reaction may be higher whereby the liquid phase is maintained during the reaction. Stirring of the mixture is continued for a short period after all the olefine has been added, whereupon the mixture is allowed to settle and the lower acid layer withdrawn on settlement, apparently little changed except in respect of colour. The clear colourless upper hydrocarbon layer after settlement is soda-washed and distilled. It is found to be almost entirely saturated, the olefine having apparently completely reacted. Some of the original iso-paraffin is recovered and can be reprocessed. When normal paraffins are present in the feed stock they too will be recovered unchanged. They should preferably be separated from the recovered unchanged iso-paraffin before re-processing the latter. The residual material has a pleasant odour and is almost entirely iso-paraffinic in composition.

In carrying out the reaction advantageously, it is desirable to employ a volume ratio of total hydrocarbon to sulfuric acid initially of between about 1.5:1 and about 2.0:1 with a calculated ratio after all of the olefin has been added of between about 2.5:1 and about 4.4:1. These ratios will be apparent from an inspection of the following examples wherein the volume ratios em-

ployed are shown to fall within these ranges. For practical purposes the ratios may be determined by computing upon the basis of volumes of isoparaffins, olefins and sulfuric acid actually employed, although it is realized that the final volumetric ratio when computed on the amount of hydrocarbon to sulfuric acid employed is not strictly accurate at the conclusion of the alkylation reaction since some olefinic reactant remains absorbed in the acid and the alkylate produced together with the unreacted hydrocarbons may possess a slightly decreased volume with respect to the initial total volumes of the reacted reactants added to the sulfuric acid. However, the ratios do provide an indication of the relative amounts of both types of reactants as well as sulfuric acid which are admixed in order to form the reaction mixture.

The following are a number of examples of the carrying out of the process of production of motor fuel according to the invention under a variety of conditions and in the use of various olefines and iso-paraffins.

#### EXAMPLE 1

Four hundred cc. of concentrated commercial sulphuric acid (approximately 97 per cent) are charged with 400 grams (about 667 cc.) of liquid isobutane at  $-12^{\circ}$  C. into a vessel fitted with an efficient stirrer and surrounded by a bath of cooling liquid maintained at  $-10^{\circ}$  C. to  $-12^{\circ}$  C. 400 grams (about 533 cc.) of diisobutene are slowly run into a mixture over a period of two hours and stirring is continued for a further period of 30 minutes after the addition of diisobutene. The volume ratio of total hydrocarbon to acid was about 1.67:1 initially and was about 3:1 or somewhat lower after all of the diisobutene had been added. The mixture is allowed to settle and the lower acid layer is run off. The acid layer is straw colored and has increased in volume by about 15 cc. The upper hydrocarbon layer is soda-washed and distilled. It boils over a comparatively wide range, and contains a considerable quantity of unreacted isobutane, the fraction  $50$ – $150^{\circ}$  C. representing 48 per cent of the total hydrocarbon charge. The portion boiling between  $90^{\circ}$  and  $110^{\circ}$  C. has an octane number of 95.5 (C. F. R. motor method). The C. F. R. motor method of determining knock-rating is described in "The Principles of Motor Fuel Preparation and Application" by Nash and Howes, vol. II, paragraph 759.

#### EXAMPLE 2

Four hundred cc. of concentrated commercial sulphuric acid (approximately 97 per cent) are thoroughly mixed with 600 cc. isopentane in a vessel surrounded by ice and fitted with a stirrer. Four hundred cc. diisobutene are added gradually over a period of two hours. The initial volume ratio of total hydrocarbon to acid was about 1.5:1. The final ratio was about 2.5:1 or actually slightly lower due to the condensation. Stirring is continued for a further period of 30 minutes after the diisobutene has been added. At the end of this time the mixture is allowed to settle and the lower acid layer is removed. The recovered acid is straw coloured and has a volume of 415 cc. approximately. The upper layer of treated hydrocarbon is soda-washed and distilled. It distills over a wide range and contains a proportion of isopentane which has not reacted. The fraction boiling from  $50$ – $175^{\circ}$  C. represented 52% of the total hydrocarbon charge and is prac-

tically completely saturated. It has an octane number of 84 (C. F. R. motor method).

#### EXAMPLE 3

5 Six hundred cc. of isopentane and 400 cc. of sulphuric acid (approximately 97 per cent) were placed in a vessel cooled in ice and the mixture vigorously stirred. When thoroughly cold 400 cc. of diisobutene were slowly added over a period of 2 hours, after which stirring was continued for a further half hour. The hydrocarbon to acid volume ratios were maintained within the ranges set forth in Example 2. The reaction product was then allowed to settle and the upper colourless hydrocarbon layer withdrawn. The acid which was a pale straw colour increased in volume in the treatment by 5–15 cc., while the volume of the hydrocarbon layer after neutralisation was approximately 875 cc., its specific gravity was .713 at  $60^{\circ}$  F., and its bromine number (Francis method) 4. The Francis method of determining bromine number is described in "The Principles of Motor Fuel Preparation and Application" by Nash and Howes, vol. II, paragraph 573. After removal by distillation of unchanged isopentane the specific gravity was .731 at  $60^{\circ}$  F., and 84 per cent boiled between 50 and  $200^{\circ}$  C. leaving a residue having a specific gravity of .789 at  $60^{\circ}$  F., and bromine number (Francis) 27. The product was fully saturated and essentially isoparaffinic in composition. The yield of the hydrocarbon boiling above  $50^{\circ}$  C. represented 176 per cent of the olefine taken. The material produced had a high antiknock rating and was produced without the application of heat and without pressure.

#### EXAMPLE 4

A polymer gasoline produced by the catalytic polymerisation of olefines and having a boiling range of  $80$ – $120^{\circ}$  C. was used as the olefinic material, having a specific gravity of .727 at  $60^{\circ}$  F., and a bromine number (Francis) of approximately 200. The treatment was carried out as in Example No. 3 using 400 cc. acid (97 per cent), 440 grams (about 730 cc.) of isobutane and 440 grams (about 587 cc.) of the polymer gasoline. The polymer gasoline was slowly added in a period of  $1\frac{1}{4}$  hours, the stirring being continued for a further  $\frac{3}{4}$  hour. The recovered acid was rather darker in colour than that recovered in Example No. 3, and had increased in volume to 450 cc. The amounts of reactants and acid correspond to an initial hydrocarbon to acid volume ratio of about 1.82:1 and a final ratio of about 3.29:1. The hydrocarbon layer after the removal of isobutane had a specific gravity of .728 at  $60^{\circ}$  F., and bromine number (Francis) 31. Fractionation yielded a product boiling over a wide range, 74 per cent boiling to  $200^{\circ}$  C., having a specific gravity of .715 at  $60^{\circ}$  F., bromine number (Francis) 21.5 and a residue having a specific gravity of .801 and bromine number (Francis) 57. The distillate boiling to  $200^{\circ}$  C. had a pleasant odour and an octane number 84.6 (C. F. R. motor method). With an addition of ethyl fluid equivalent to 2 cc. tetra ethyl lead per (Imp.) gal. the octane number was raised to 95.5. It may be noted that while the bromine number of the fractionated reaction product was high, the bromine number of the polymer gasoline was very high, and that modification of conditions would have resulted in an even lower bromine number of the fractionated product.

## EXAMPLE 5

Sixteen hundred cc. of sulphuric acid (97 per cent) were placed in a pressure vessel provided with a stirrer and an external jacket through which cold or warm kerosene or the equivalent could be circulated, and 1800 grams (about 3210 cc.) of isobutane were added. The acid and paraffin were then stirred with warm kerosene circulating through the jacket, until the temperature of the mixture reached 20° C., the pressure reaching 45 lb. per sq. inch (gauge), when 1800 grams (about 2490 cc.) of diisobutene were slowly added with vigorous stirring. Cooled kerosene was circulated through the jacket during this addition to remove the heat evolved, so maintaining the temperature of the mixture at about 20° C. The addition required 1½ hours, after which stirring was continued for a further ½ hour. The pressure had then fallen to about 10–15 lb. per sq. inch (gauge). The hydrocarbon to acid ratios were initially about 2:1 and finally about 3.56:1.

To facilitate handling, the product was then cooled down to 0° C., the acid and hydrocarbon

jected to a cracking distillation may first be treated in known manner with sulphuric acid (60 per cent) followed by heating and polymerisation whereby there is produced a mixture of diisobutene and triisobutene in addition to a proportion of unchanged material. The diisobutene and triisobutene may be subjected to contact with an isoparaffin in the presence of sulphuric acid as hereinbefore described.

Alternatively the mixture of diisobutene and triisobutene may be fractionated and the diisobutene may be hydrogenated by known means to produce an iso-octane of 100 octane number, and the triisobutene may be subject to contact with an iso-paraffin in the presence of sulphuric acid as hereinbefore described for the production of a saturated spirit of high anti-knock value having an octane number of about 89 to 90.

From the product of the reaction of isobutane and isobutene or polyisobutene, iso-octane, (2.2.4 trimethylpentane) may be separated by fractionation. Among other hydrocarbons which may be isolated by fractionation are: 2-methylbutane (isopentane), 2,3 dimethylbutane, 2,3- and 2,4-dimethylpentane and 2,2,5 trimethylhexane.

TABLE NO. 1

Tabulated examples of treatments carried out according to the invention in which the following olefins, viz: (i) diisobutene, (ii) triisobutene and (iii) propylene were used with isobutane, in each case in the following proportion:

|                                                                                              |           |
|----------------------------------------------------------------------------------------------|-----------|
| Sulphuric acid (approximately 97% except in run No. 5 in which the acid strength was 100.6%) | cc.. 1600 |
| Isobutane                                                                                    | g.. 1800  |
| Olefin (i) or (ii)                                                                           | g.. 1800  |
| Olefin (iii)                                                                                 | g.. 1300  |

| Run No. | Olefin | Temp., °C. | Per cent product >27° C. on olefin taken | Boiling range of product: 27–185° C. |             |              |                              |      | Residue >185°                           |                          |             |              |
|---------|--------|------------|------------------------------------------|--------------------------------------|-------------|--------------|------------------------------|------|-----------------------------------------|--------------------------|-------------|--------------|
|         |        |            |                                          | Per cent on olefin taken             | Bromine No. | S. G./60° F. | Engine test                  |      |                                         | Per cent on olefin taken | Bromine No. | S. G./60° F. |
|         |        |            |                                          |                                      |             |              | 50% in H. O. S. <sup>1</sup> | Neat | +1½ cc. tetraethyl lead per (Imp.) gal. |                          |             |              |
| 1.      | (i)    | -10        | 152                                      | 106                                  | <1          | .709         | 72.9                         | 92.1 | 105                                     | 36.4                     | 22          | .786         |
| 2.      | (i)    | +20        | 158                                      | 133                                  | <1          | .710         | 70.5                         | 89.3 | 99.7                                    | 20                       | 13.5        | .781         |
| 3.      | (ii)   | -10        | 152                                      | 106                                  | <1          | .710         | 71.2                         | 88.8 | 100.6                                   | 38.1                     | 33          | .792         |
| 4.      | (ii)   | +20        | 163                                      | 138                                  | <1          | .704         | 68.9                         | 88.7 | 98.9                                    | 20.5                     | 13          | .782         |
| 5.      | (iii)  | 25–30      | 150                                      | 122                                  | <1          | .698         | 67.4                         | 82.5 | 93.3                                    | 23.0                     | 2.5         | .776         |

<sup>1</sup> Basic blending material, 52.5 octane number.

layers separated, and the hydrocarbon layer completely neutralised with soda. The results of the treatment in the use of diisobutene as olefinic material and isobutane as the paraffin are recorded below in run No. 2 of Table No. 1, together with the results of similar runs when using triisobutene under the same conditions (runs 3 and 4—Table No. 1).

Similar results are obtained when operating at +30° C. although there is a little more SO<sub>2</sub> formation than at the lower temperature. The acid however retains the same appearance.

By operating at -10° C. a somewhat lower yield of useful product, that is a fraction having a boiling range of 27–185° C. is obtained, but this possesses a slightly higher octane rating (runs 1 and 3—Table No. 1). The efficiency of the agitation is an important factor, the product improving with increasing efficiency of agitation.

The acid in these runs is not spent and may be used repeatedly or employed for other refining operations.

Isobutene may be used instead of or together with diisobutene or triisobutene or other such olefines or mixtures of diisobutene and triisobutene may be used.

Thus in carrying out the process, gases from a cracking plant in which a petroleum stock is sub-

50 TABLE NO. 2  
A. S. T. M. (American Standard Test Method)  
distillations of the products of runs 2, 4 and 5  
referred to in Table No. 1

|                            |                            | Run 2 | Run 4 | Run 5 |
|----------------------------|----------------------------|-------|-------|-------|
| 55                         | Initial boiling point, °C. | 43    | 32    | 43.5  |
| 2%                         |                            | 64    | 44    | 59.5  |
| 5%                         |                            | 77.5  | 55    | 69    |
| 10%                        |                            | 90    | 69    | 80    |
| 20%                        |                            | 102   | 93.5  | 90    |
| 30%                        |                            | 110   | 105   | 98    |
| 40%                        |                            | 115.5 | 111   | 101.5 |
| 50%                        |                            | 120.5 | 122   | 109   |
| 60%                        |                            | 129   | 131   | 122   |
| 70%                        |                            | 140   | 143.5 | 145.5 |
| 80%                        |                            | 162   | 167   | 169.5 |
| 90%                        |                            | 196.5 | 198   | 200   |
| 65 Final boiling point     |                            | 257   | 244   | 248   |
| Total distillate, per cent |                            | 98    | 98    | 97.5  |
| Residue                    |                            | 1     | 1     | 1     |
| Loss                       |                            | 1     | 1     | 1.5   |
| Vol. to 70° C., per cent   |                            | 3     | 10.5  | 5.5   |
| 100°                       |                            | 19    | 25    | 36.5  |
| 140°                       |                            | 70    | 67    | 67    |

In run No. 5 of Table No. 1 the reaction between isobutane and propylene was conducted in the same way as with isobutane and diisobutene. Propylene was added as liquid under pressure and sulphuric acid containing 2.5% free

sulphur trioxide (equivalent to 100.6% sulphuric acid) was used. At the end of the reaction the pressure fell practically to that of the atmosphere on cooling the vessel to 0° C.

Inasmuch as when using propylene a small amount of dialkyl sulphate is present in the hydrocarbon layer, neutralisation should be thoroughly carried out (as for example by stirring with 10 per cent soda for 5 hours) to prevent the formation of free acid and acid products with consequent charring of the contents of the still during the subsequent distillation.

relatively little disadvantage since it can be easily recovered by distillation and re-used.

By "substantial or considerable excess" is meant a substantially greater excess of isobutane than that small excess required to ensure against the momentary presence in the vigorously stirred reaction mixture of a local excess of the olefine as it is slowly added and admixed with isobutane or isopentane and sulphuric acid during the period of contact, which substantially greater excess may reach a considerable proportion with the practical advantages referred to.

TABLE NO. 3

Tabulated results of two experiments carried out according to the invention in which the isobutane:diisobutene ratios by weight were respectively 1:1 and 2:1.

Diisobutene and isobutane at 20° C. using 96.9 per cent acid  
Pressure used sufficient to maintain the isobutane in the liquid phase

Time of addition: 90 min. Time of stirring: 30 min.

Expt. No. 1.—1:1 3000 cc. isobutane Expt. No. 2.—2:1 4500 cc. isobutane  
1800 g. diisobutene 1350 g. diisobutene  
(2490 cc.) (1875 cc.)

Ratio hydrocarbon:acid Initial 1.88:1 Ratio hydrocarbon:acid Initial 3.75:1  
Final 3.44:1 Final 5.3:1

| Isobutane:diisobutene ratio | Volume acid taken | Per cent on olefine taken | Product >27° C.          |         |    |     |       |       |       |       |       |     |     |      | Product 27-185° C. |                |               |                           |             |                     | Residue         |      |                   |                           |
|-----------------------------|-------------------|---------------------------|--------------------------|---------|----|-----|-------|-------|-------|-------|-------|-----|-----|------|--------------------|----------------|---------------|---------------------------|-------------|---------------------|-----------------|------|-------------------|---------------------------|
|                             |                   |                           | A. S. T. M. distillation |         |    |     |       |       |       |       |       |     |     |      | Engine test        |                |               |                           |             |                     |                 |      |                   |                           |
|                             |                   |                           | I. B. P., ° C.           | 2%      | 5% | 10% | 20%   | 30%   | 40%   | 50%   | 60%   | 70% | 80% | 90%  | F. B. P., ° C.     | Per cent T. D. | Per cent res. | Per cent on olefine taken | Bromine No. | Sp. gr. at 15.6° C. | 50% in H. O. S. | Neat | Neat+1.5 cc. TEL. | Per cent on olefine taken |
| 1:1                         | 1,600             | 165                       | 38.45.5                  | 53.66.5 | 94 | 105 | 112.5 | 117.5 | 125.5 | 137.5 | 160.5 | 197 | 257 | 97.5 | 1.5                | 136            | <1            | .705                      | 71.2        | 90.5                | 98              | 22   | 14                | .783                      |
| 2:1                         | 1,200             | 184                       | 33.39                    | 49.64   | 89 | 101 | 107   | 112   | 118.5 | 128   | 148   | 194 | 230 | 96.5 | 1                  | 158            | <1            | .700                      | 71.1        | 91.3                | 98.9            | 14.8 | 9.5               | .782                      |

The product from this reaction contains considerable quantities of 2.3- and 2.4-dimethylpentanes.

## EXAMPLE 6

In the foregoing examples the proportion of the isoparaffin to olefine is approximately such that for each molecule of the former one molecule of the latter or its equivalent in the case of polymerides is taken. Since the polymerides so far examined behave as though depolymerised to the monomeric form before reaction, the quantity of iso-paraffin required is determined by the monomeric equivalent of the polymer, e. g. two molecular proportions of iso-butane to one of diisobutene, three molecular proportions of isobutane to one of triisobutene and so on. The proportion indicated in the foregoing examples are not however essential. On the contrary substantial or considerable excess of the iso-paraffin or iso-paraffins is generally advantageous in point of overall yield of the product, high proportion of useful material in the product and the lower boiling range of the small residue obtained. These advantages were demonstrated in the results recorded in the following Table No. 3 which were obtained with diisobutene and isobutane in the weight ratios of 1:1 and 1:2. The results recorded in Table No. 3 indicate that a substantial or considerable excess of iso-butane favours the formation of the octane fraction. The proportion of useful product is much higher than when equimolecular proportions of isobutane and olefine are used. The yield of 2.2.4 trimethylpentane recoverable by distillation is also increased considerably. Similar results were obtained in the use of triisobutene in place of the dimeride. On the other hand the use of isobutane in substantial or considerable excess offers

## EXAMPLE 7

To 3000 cc. isobutane and 1600 cc. of sulphuric acid (97 per cent) were added while maintaining the temperature at 20° C., 2250 cc. of liquid butene-2 during a period of 1½ hours and sufficient pressure was applied to maintain the liquid phase. After agitating for a further ½ hour, the product was separated and worked up as in previous examples. The initial volume of hydrocarbon to acid ratio was about 1.87:1 while the final ratio was about 3.28:1. The overall yield of product based upon the olefine taken was 164 per cent, the specific gravity of the product .706 at 60° F. and the bromine number (Francis) 3. On distillation the yield of the fraction having the boiling range 27-185° C. was equivalent to 148 per cent of the olefine taken. This fraction had a specific gravity of .706 at 60° F., bromine number (Francis) less than 1, and an octane rating of 90.2 octane number increasing to 100.3 octane number on addition of ethyl fluid equivalent to 1.5 cc. tetra ethyl lead per gallon (Imp.). The distillation range of the product was substantially the same as that obtained when diisobutene is used under similar conditions. Fractionation indicated the presence of appreciable quantities of iso-octane (2.2.4 trimethylpentane) in this product.

## EXAMPLE 8

The olefine employed consisted in a fraction having a boiling range of 105-112° C. taken from the product formed by the condensation of n-butene and isobutene in the C<sub>4</sub> cut from gas derived from an oil cracking plant, when using a phosphoric acid catalyst. The material in question consisted largely of the condensation product from one molecule each of n-butene and isobutene, being essentially a 2.2.3, trimethylpentene,

and is hereinafter referred to as butene-isobutene polymer.

To a mixture of 1600 cc. sulphuric acid (97 per cent) and 3000 cc. isobutane were added 1800 g. (about 2430 cc.) of butene-isobutene polymer over a period of 90 minutes maintaining the temperature steady at 20° C. against the heat of condensation, the pressure being sufficient to maintain the liquid phase. Finally, after a further 30 minutes agitation, the product was separated from the acid and worked up as in previous examples. The initial hydrocarbon to acid ratio was about 1.87:1 with a final ratio of about 3.4:1. The yield of the crude product of specific gravity .713 at 60° F. and bromine number (Francis) 2, was equivalent to 158 per cent yield based upon the olefine taken. On distillation the yield of the fraction having a boiling range of 27-185° C. was equivalent to 135% of the olefine taken. This fraction had a specific gravity .707 at 60° F., bromine number (Francis) less than 1 and an octane rating of 87, the octane number increasing to 97.9 with addition of ethyl fluid equivalent to 1.5 cc. tetra ethyl lead per gallon (Imp.).

The product obtained from a crude butene-isobutene polymer, a fraction of boiling range 95-120° C. which also contained a small amount of diisobutene gave practically the same yield, but the octane rating of the product was 88.7 octane number, and 99.2 octane number with addition of 1.5 cc. tetra ethyl lead per gallon (Imp.).

#### EXAMPLE 9

To 2000 cc. isobutane and 1070 cc. of sulphuric acid (97 per cent) were added while maintaining the temperature at 20° C. and stirring vigorously, 2700 cc. of a crude C<sub>4</sub> fraction cut from cracking gas and containing 94% of C<sub>4</sub> unsaturated hydrocarbons, the pressure used being sufficient to maintain the reactants in the liquid phase. Addition was carried out over a period of 90 minutes followed by a further 30 minutes agitation. The initial hydrocarbon to acid volume ratio was about 1.87:1 with the final ratio being roughly 4.4:1. The crude product after a thorough neutralisation with caustic soda was redistilled and yielded a fraction boiling 27-185° C. with a gravity of .706/60° F. and bromine number (Francis) of 1. Tested on the engine the neat product gave by the C. F. R. motor method 91.6 octane number rising to 99.5 octane number with the addition of ethyl fluid corresponding to 1.5 cc. tetraethyl lead per (Imp.) gal.

It will be understood that the process may be advantageously carried out continuously, and that instead of sulphuric acid being used phosphoric acid may be used alone or with sulphuric acid in the process.

We claim:

1. A process which comprises condensing at least one isoparaffin with at least one olefin in the presence of concentrated sulfuric acid while correlating the reaction conditions to produce a normally liquid, substantially completely saturated product, the volumetric ratio of the total hydrocarbon present in the reaction zone to the amount of sulfuric acid present therein being maintained between about 1.5:1 and about 4.4:1.

2. A process which comprises reacting low boiling olefins with low boiling isoparaffins, the isoparaffins being present in the reaction mixture throughout the entire reaction in substantial molar excess over the stoichiometrical equivalent monomeric contents of the olefins in the presence of concentrated sulfuric acid while maintaining

alkylating reaction conditions and a volume ratio of total quantities of hydrocarbons to sulfuric acid in the reaction zone of between about 1.5:1 and about 4.4:1.

3. A process as in claim 2 wherein the reacting mixture is maintained substantially in the liquid phase throughout the reaction.

4. A process for the production of normally liquid, saturated hydrocarbons boiling substantially within the motor fuel gasoline boiling range which comprises reacting isobutane with diisobutylene, the isobutane being present in at least 2 mols per mol of diisobutylene, at a temperature of between about -10° C. and about +20° C. under sufficient superatmospheric pressure to maintain the reactants in the liquid phase, in the presence of concentrated sulfuric acid, maintaining vigorous agitation of the reaction mixture, maintaining a volumetric ratio of total hydrocarbon to acid in the reaction zone of from about 1.5:1 to about 4.4:1, for a length of time sufficient to effect a substantial alkylation reaction, and recovering the normally liquid saturated product from the reaction mixture.

5. A process as in claim 4 wherein the process is carried out continuously.

6. A process as in claim 4 wherein the diisobutylene is substituted by a polymer gasoline prepared by condensing olefins having no more than 4 carbon atoms per molecule.

7. A process for the production of normally liquid, substantially completely saturated hydrocarbons boiling within the gasoline boiling range which comprises condensing isobutane with monoolefins having fewer than five carbon atoms per molecule, the isobutane being present in substantial molar excess of the olefins present in the liquid phase, with vigorous agitation, at a temperature between about -10° C. and about +20° C., in the presence of concentrated sulfuric acid and for sufficient length of time to effect substantial alkylation, the hydrocarbon to sulfuric acid volume ratio being maintained between about 1.5:1 and about 4.4:1 in the reaction mixture, and recovering the reaction products from the reacted mixture.

8. A process as in claim 7 wherein C<sub>4</sub> monoolefins are employed and the reaction is carried out continuously.

9. A process for the production of normally liquid, saturated, branched chain hydrocarbons which comprises reacting isoparaffin with liquid monoolefin in the presence of concentrated sulfuric acid of alkylating strength with vigorous agitation under alkylation reaction conditions and under sufficient superatmospheric pressure to maintain liquid phase operation while maintaining a hydrocarbon:acid volume ratio between about 1.5:1 and about 4.4:1.

10. A process as in claim 9 wherein the olefin is added gradually with agitation to a pre-adixture of the isoparaffin and the sulfuric acid and wherein the isoparaffin is maintained in substantial molar excess over the olefin throughout the reaction.

11. A process for the production of motor fuel constituents comprising essentially branched chain, saturated hydrocarbons boiling within the motor fuel range which comprises reacting a liquid monoolefin with at least one isoparaffin in the presence of 97-100% sulfuric acid under alkylation reaction conditions wherein the total hydrocarbon:acid volume ratio is maintained between about 1.5:1 and about 4.4:1.

12. A process which comprises maintaining a

liquid admixture comprising essentially at least one paraffinic hydrocarbon containing at least one tertiary carbon atom per molecule and sulfuric acid having a concentration between about 97% and about 100% in a volume ratio of between about 1.5:1 and about 2:1, maintaining said mixture under alkylation reaction conditions, alkylating the isoparaffin content thereof by adding gradually to the mixture monoolefin while agitating the reaction mixture, the total hydrocarbon:acid ratio being maintained during the reaction between about 2.5:1 and about 4.4:1.

13. A process which comprises condensing at least one isoparaffin with at least one normally liquid olefinic polymer in the presence of concentrated sulfuric acid of alkylating strength under alkylation reaction conditions while maintaining the volumetric ratio of total hydrocarbon to total sulfuric acid between about 1.5:1 and about 4.4:1.

14. A process as in claim 13 wherein the volumetric ratio is maintained initially between about 1.5:1 and about 2.0:1 and finally from between

about 2.5:1 and about 4.4:1 and wherein the isoparaffin is in substantially molar excess over the olefin.

15. A process for the production of normally liquid isoparaffinic hydrocarbons boiling within the motor fuel range which comprises reacting at least one isoparaffin with at least one normally liquid olefin polymer at a temperature between about -10° C. and about +30° C. under at least sufficient superatmospheric pressure to maintain the reactants substantially completely in the liquid phase, in the presence of sulfuric acid of about 97% concentration, the hydrocarbon to acid volumetric ratio being maintained between about 1.5:1 and about 4.4:1, while maintaining the reaction mixture intensively agitated for a length of time sufficient to effect a substantial alkylation reaction and recovering from the reacted mixture the isoparaffinic constituents of the desired boiling range.

ALBERT ERNEST DUNSTAN.  
STANLEY FRANCIS BIRCH.